



US011878344B2

(12) **United States Patent**  
Ma et al.

(10) **Patent No.:** US 11,878,344 B2  
(45) **Date of Patent:** Jan. 23, 2024

(54) **DIRECTIONALLY SOLIDIFIED HIGH-BORON AND HIGH-VANADIUM HIGH-SPEED STEEL AND METHOD FOR PREPARING SAME**

(71) Applicant: **XI'AN JIAOTONG UNIVERSITY**, Xi'an (CN)

(72) Inventors: **Shengqiang Ma**, Xi'an (CN); **Ping Lv**, Xi'an (CN); **Pengjia Guo**, Xi'an (CN); **Jiandong Xing**, Xi'an (CN); **Xu Tan**, Xi'an (CN); **Shasha Fu**, Xi'an (CN)

(73) Assignee: **XI'AN JIAOTONG UNIVERSITY**, Xi'an (CN)

(\*) Notice: Subject to any disclaimer, the term of this patent is extended or adjusted under 35 U.S.C. 154(b) by 15 days.

(21) Appl. No.: **17/836,242**

(22) Filed: **Jun. 9, 2022**

(65) **Prior Publication Data**

US 2022/0297180 A1 Sep. 22, 2022

(51) **Int. Cl.**

**B22D 27/04** (2006.01)  
**C22C 38/02** (2006.01)  
**C22C 38/04** (2006.01)  
**C22C 38/06** (2006.01)  
**C22C 38/22** (2006.01)  
**C22C 38/28** (2006.01)  
**C22C 38/32** (2006.01)  
**C21C 7/06** (2006.01)  
**C22C 33/06** (2006.01)

(Continued)

(52) **U.S. Cl.**

CPC ..... **B22D 27/045** (2013.01); **C21C 7/06** (2013.01); **C22C 33/06** (2013.01); **C22C 38/02** (2013.01); **C22C 38/04** (2013.01); **C22C 38/06** (2013.01); **C22C 38/22** (2013.01); **C22C 38/24**

(2013.01); **C22C 38/28** (2013.01); **C22C 38/32** (2013.01); **B22D 29/00** (2013.01)

(58) **Field of Classification Search**

CPC ..... B22D 27/045; C21C 7/06; C22C 38/22; C22C 33/06

See application file for complete search history.

(56)

**References Cited**

U.S. PATENT DOCUMENTS

3,437,131 A \* 4/1969 Ornitz ..... B22D 13/102  
164/33  
2015/0299817 A1 \* 10/2015 Shimotsu ..... C21D 8/0294  
148/566

FOREIGN PATENT DOCUMENTS

CN 101078090 \* 11/2007  
CN 100405510 \* 7/2008  
CN 101240402 A 8/2008

(Continued)

OTHER PUBLICATIONS

"Quenching Media" ASM Handbooks, vol. 4 1991, p. 67-120 (Year: 1991).\*

(Continued)

*Primary Examiner* — Nicholas A Wang

(57) **ABSTRACT**

Disclosed are a high-boron high-vanadium high-speed steel and a method for preparing the same. Pig iron, scrap steel, ferrochromium, ferromanganese, ferroboron, ferrovanadium, industrial pure iron, ferromolybdenum, ferrotungsten, ferrosilicon and ferrotitanium are subjected to smelting at 1580-1600° C. and refining to obtain a liquid steel. The liquid steel is subjected to superheating, and directional solidification at a casting temperature of 1420-1430° C., and cooled to room temperature to obtain the directionally solidified high-speed steel.

**7 Claims, 4 Drawing Sheets**



(51) **Int. Cl.**  
*C22C 38/24* (2006.01)  
*B22D 29/00* (2006.01)

(56) **References Cited**

FOREIGN PATENT DOCUMENTS

|    |             |   |         |
|----|-------------|---|---------|
| CN | 102366830   | * | 3/2012  |
| CN | 102626771   | * | 8/2012  |
| CN | 108359916 A |   | 8/2018  |
| CN | 108842116   | * | 11/2018 |
| CN | 111074142 A |   | 4/2020  |
| GB | 842951 A    |   | 7/1960  |

OTHER PUBLICATIONS

Zhou Chenming, Li Yefei, Yi Dawei, Ma Shengqiang, Liu Hong-gang; Study on abrasive wear properties of the directional solidified Fe-B casting alloy; China Foundry Machinery & Technology, vol. 54 No. 5, Sep. 2019; State Key Laboratory for Mechanical Behavior of Materials, Xi'an Jiaotong University, Xi'an 710049, Shaanxi China.

\* cited by examiner



Fig. 1



Fig. 2a



Fig. 2b



Fig. 2c



Fig. 2d



Fig. 2e



Fig. 2f



Fig. 3



Fig. 4

## 1

**DIRECTIONALLY SOLIDIFIED  
HIGH-BORON AND HIGH-VANADIUM  
HIGH-SPEED STEEL AND METHOD FOR  
PREPARING SAME**

**CROSS-REFERENCE TO RELATED  
APPLICATIONS**

This application claims the benefit of priority from Chinese Patent Application No. 202110925617.4, filed on Aug. 12, 2021. The content of the aforementioned application, including any intervening amendments thereto, is incorporated herein by reference in its entirety.

**TECHNICAL FIELD**

This disclosure relates to the manufacturing of directionally solidified wear-resistant metal materials, and more particularly to a directionally solidified high-boron and high-vanadium high-speed steel and a method for preparing the same.

**BACKGROUND**

High-speed steel has been widely used as a wear-resistant metal material and tool steel. It is mainly composed of metal matrix and hard-phase carbides distributed over the metal matrix. The hard-phase carbides can enhance the wear resistance of the high-speed steel as the strengthening constitutes, and the metal matrix as a toughening phase contributes excellent stiffness and shock absorption to the high-speed steel. The high-speed steel is a heavily alloyed material, in which vanadium has a significant effect on the microstructure and properties of high-speed steel. For instance, vanadium can facilitate the formation of MC-type carbides and lamellar M<sub>2</sub>C-type carbides, and inhibit the formation of skeletal M<sub>6</sub>C-type carbides to enhance the wear resistance of the high-speed steel. The orientation of the hard phase (e.g., carbides or borides in steels) will significantly affect the overall performance of the metal material. Even for the same material, different hard phase orientations may alter the overall performance of the alloy. When suffering friction and wear, the change in the orientation of the wear-resistant phase in metal material will greatly alter the wear resistance of the material and other properties.

The matrix microstructure of the high-boron high-speed steel is usually composed of a martensitic matrix, on which a large number of high-hardness borocarbides or eutectic borides are distributed in a network. The high-boron high-speed steel has a high hardness owing the presence of these eutectic borides. Nevertheless, considering that the eutectic borocarbides or borides has large inherent brittleness and coarse morphology and size, and is distributed in a network on the matrix, the high boron high-speed steel is naturally brittle and hard, and thus the rolls manufactured therefrom are prone to peeling, cracking and wear.

**SUMMARY**

An object of the present disclosure is to provide a directionally solidified high-boron high-vanadium high-speed steel and a method for preparing the same to overcome deficiencies in the prior art. The method provided herein realizes the effective regulation to control of the size, shape and distribution of the borides and carbides in the high-speed steel, which can simultaneously achieve the desired microstructural orientation and the tailored strengthening

## 2

and toughening of the high-boron high speed steel, as well as the coordination between the special microstructure orientation and excellent unique properties, greatly enhancing the service life and performance. This application offers a new idea and insight for developing wear-resistant high-boron high-speed steels.

Technical solutions of this disclosure are described as follows.

In a first aspect, this disclosure provides a method of preparing a directionally solidified high-speed steel, comprising:

(S1) subjecting a raw material to smelting at 1580-1600° C. and refining to obtain a liquid steel; wherein the raw material comprises pig iron, scrap steel, ferrochromium, ferromanganese, ferroboron, ferrovanadium, industrial pure iron, ferromolybdenum, ferrotungsten, ferrosilicon and ferrotitanium; and

(S2) subjecting the liquid steel to superheating and directional solidification at a casting temperature of 1420-1430° C. followed by cooling to room temperature to obtain the directionally solidified high-speed steel.

In some embodiments, in step (S1), the raw material comprises 4.893-4.894% by weight of the pig iron, 25.176-25.177% by weight of the scrap steel, 8.520-8.521% by weight of the ferrochromium, 1.038-1.039% by weight of the ferromanganese, 10.899-10.900% by weight of the ferroboron, 4.148-4.149% by weight of the ferrovanadium, 41.850-41.860% by weight of the industrial pure iron, 1.121-1.122% by weight of the ferromolybdenum, 1.554-1.555% by weight of the ferrotungsten, 0.463-0.464% by weight of the ferrosilicon and 0.335-0.336% by weight of the ferrotitanium.

In some embodiments, in step (S1), the smelting and the refining are performed through steps of:

feeding the scrap steel, the pig iron and the industrial pure iron to a furnace, and then feeding the ferromolybdenum, the ferrochromium, the ferrotungsten, the ferrovanadium, the ferromanganese and the ferrosilicon to the furnace; heating the furnace to 1550-1600° C. to obtain a first melt; transferring the first melt to a ladle; feeding the preheated ferroboron and the ferrotitanium to the furnace and then transferring the first melt in the ladle back to the furnace to obtain a second melt; transferring the second melt to the ladle; introducing 0.148-0.152 g of an aluminum filament to a bottom of the furnace for deoxidization; transferring the second melt with the desired chemical composition requirements back to the furnace; and performing argon blowing at the bottom of the furnace for 8-15 min for refining.

In some embodiments, the directional solidification is performed in a directional solidification device equipped with a sodium silicate-bonded sand mold as a cast mould; an inner side surface of the sodium silicate-bonded sand mold is coated with an aluminum oxide coating with an average thickness of 0.8-1.1 mm so as to prevent side wall heat dissipation.

In some embodiments, in step (S2), before the directional solidification, the sodium silicate-bonded sand mold is dried at 250-280° C. for 6-8 h.

In some embodiments, in step (S2), the superheating of the liquid steel is performed at 1510-1520° C. for 10-12 min with a superheat degree of 49.8-50.2° C.

In some embodiments, in step (S2), a top end of a casting riser of the directional solidification device is spread with a thermal insulating agent to maintain the thermal insulation; thus, according to the directional solidification device mentioned above, the whole directional solidification device can ensure a Y-type ingot (as shown in FIG. 1) with a heat

dissipation producing a one-way heat extraction established as the strong heat gradient from casting mould to a chiller creating a cooling condition; the directional solidification is performed at a cooling rate of 12.1-12.3° C/s for 19.0-21.0 s; and after the Y-type ingot is cooled to room temperature, the directionally solidified high-speed steel is subjected to mold dismantling, shakeout and wire cutting.

In some embodiments, the directional solidification device adopts a thermal-couple for heating monitor, and a pure ion block embedded with a copper block as a chiller for cooling.

In some embodiments, the casting mould of the directional solidification device is coated with the aluminum oxide coating layer having a thickness of 0.8-1.1 mm.

In a second aspect, this disclosure provides a directionally solidified high-boron high-vanadium high-speed steel, comprising:

- a metal matrix; and
- a hard-phase boride distributed on the metal matrix;
- wherein the directionally solidified high-speed steel consists of 0.35-0.48% by weight of C, 1.77-1.82% by weight of B, 4.76-4.81% by weight of Cr, 0.58-0.73% by weight of Si, 0.64-0.90% by weight of Mn, 1.19-1.23% by weight of W, 0.63-0.67% by weight of Mo, 0.06-0.10% by weight of Ti, 0.59-0.61% by weight of Al, 1.88-2.30% by weight of V, balance with Fe and trace impurities.

Compared with the prior art, the beneficial effects of the present disclosure are described below.

With respect to the method provided herein for preparing a directionally solidified high-boron high-vanadium high-speed steel, the sodium silicate-bonded sand mold is subjected to drying and thermal insulation prior to the casting, and the raw materials are subjected to smelting, refining and thermal insulation treat of the liquid steel (namely melt). In this way, individual phases in the steel are refined, and various defects and inclusions in the casting process can be alleviated or almost eliminated. Moreover, the yield of casting elements is improved. The casting and directional solidification of the purified melt in the directional solidification device is subject to one-way heat extraction as the thermal conductivity control to obtain the excellent casting or ingot with dense and fine microstructure while ensuring that the casting microstructure is orderly arranged along the solidification direction. As a result, the grain orientation of the microstructure is well controlled, and the distribution of the columnar grains and grain boundary is optimized. The casting prepared by the method of the disclosure has excellent resistance to thermal shock and oxidation, extended fatigue life and desired resistance to high temperature creep. In order to promote the directional microstructure in the steel, the vanadium-boron composition design, melt super-heating treatment, refinement, and control and monitor the one-way heat extraction of directional solidification are integrated. With respect to the resulting directionally solidified high-boron high-vanadium high-speed steel, the micro-hardness of the boride increases with the increase of vanadium content in different crystal growth orientations of borides. In particular, in the presence of 2.05 wt. % vanadium, the bulk hardness of directionally solidified high-boron high-vanadium high-speed steel in the growth plane of the borides (namely  $M_2B$  boride (002) plane as its preferred growth plane) reaches the maximum value of 62.1 HRC, which is 13.04% higher than that of the as-cast ordinary solidification high-boron high-speed steel, and 35.42% higher than that of the as-cast ordinary solidification high-boron high-speed steel bearing 0.4% by weight of C, 2.0% by weight of B, and 1.0% by weight of V (e.g., 40.1

HRC). At the same time, the toughness of the directionally solidified high-boron high-vanadium high-speed steel is improved by 32%. In addition, the bending strength of the directionally solidified high-boron high-vanadium high-speed steel is also enhanced with the increase of the vanadium content, and when the vanadium content is 2.05 wt. %, the bending strength of the directionally solidified high-boron high-vanadium high-speed steel parallel to the preferred growth orientation (i.e.,  $Fe_2B$  or  $M_2B$  [002] orientation) reaches the maximum 1724 MPa, which is 12.41% higher than that of the as-cast ordinary solidification high-speed steel.

By regulating the raw material composition, a high-boron high-vanadium high-speed steel casting with 1.88-2.30% by weight of vanadium and other elements meeting the specifications can be obtained, which has enhanced strength and toughness. In the case of increased vanadium content and lowered boron content, the fracture strength, toughness and orientation effect are simultaneously enhanced.

The scrap steel, pig iron and industrial pure iron are fed to the furnace ahead of the ferromolybdenum, ferrochromium, ferrotungsten, ferrovaniadium, ferromanganese and ferrosilicon to form a first melt, and the melting temperature and reaction time of the liquid steel containing various several elements are adjusted to control the compositional content of the liquid steel to a reasonable range. After that, the first melt is transferred to a ladle, and simultaneously, the pre-heated ferroboron and ferrotitanium are fed to the bottom of furnace to be molten uniformly. Subsequently, the first melt in the ladle is transferred to the furnace to obtain a second melt, and the second melt is transferred to the ladle. When the second melt in the ladle is close to 1520-1530° C., some aluminum filaments are fed to the bottom of the furnace for deoxidization, and then the second melt in the ladle is transferred back to the furnace. Argon blowing is performed at the bottom of the furnace to remove oxides and other inclusion impurities in the second melt to enable the refinement and purification, eliminating the casting defects and controlling the metallurgical quality. In the method provided herein, the smelting process is performed at 1580-1600° C., higher than the melting point of iron (1534° C.), so that the raw materials can be molten rapidly to ensure the full stirring and melting, enhancing the refinement and purification effect.

Further, the coating layer of the casting mold is 0.8-1.1 mm in thickness, which can mitigate the thermal impact of the high-temperature liquid steel on the casting mold and reduce the internal stress of the arm, preventing the casting from cracking. Moreover, the coating layer with such thickness can also play an important role in improving the heat insulation which ensure the one-way heat extraction as the thermal conductivity control to avoid the heat dissipation of the side wall of the mold.

Before the casting, the sodium silicate-bonded sand mold is dried at 250-280° C. for 6-8 h to prevent the gas evolution during the casting, avoiding the defects in the casting such as strength decline and pores. In this case, when the liquid steel is poured into the cavity formed by the directional solidification device, the side of the cavity hardly affects the heat dissipation, and finally a strong unidirectional heat dissipation condition is formed from top to bottom.

Further, the molten high-boron high-vanadium high-speed steel is kept at 1510-1520° C., higher than the melting point of iron, for 10-12 min to stay liquid and reach the complete mixing and uniform distribution of various elements, which facilitates avoiding the segregation. Furthermore, the casting temperature is 1410-1440° C., slightly

higher than the liquidus temperature (1381° C.) in the phase diagram of the Fe—B alloy, which can maintain a certain degree of superheat to ensure the casting quality.

Further, in the presence of a thermal insulating agent, the cooling of the casting is accelerated, and a desired temperature gradient is reached to form the ideal directionally solidified columnar crystal microstructure and enable the good filling, the excellent feeding conditions and the easy healing of thermal crack, facilitating the manufacturing of dense and sound castings.

Further, a composite cooling system, formed by a pure ion block and a small square copper block closely embedded in the bottom thereof, is employed in the directional solidification device, which accelerates the cooling of the casting and offers the desired temperature gradient to form the ideal directionally solidified columnar crystal microstructure.

The directional solidification technique is performed at a cooling rate of 12.1-12.3° C./s for 19.0-21.0 s to ensure the good filling capacity, excellent feeding conditions and easy healing of the thermal crack, such that the obtained casting is dense and sound. Additionally, the coating layer of the directional solidification device is set to 0.8-1.1 mm in thickness, which can alleviate the heat impact of the high-temperature liquid steel on the casting mold and reduce the internal stress of the arm, preventing the obtained casting from cracking. The coating layer also strongly contributes to the heat insulation and the improvement of the filling performance of the casting mold.

The boron and vanadium-bearing high-speed steel provided in this application has a good orientation effect, in which a columnar dendritic microstructure is formed, and the horizontal grain boundary is eliminated, improving the resistance to high temperature creep and fatigue. When the vanadium content is 2.05 wt. %, the alloy has an evenly distributed hard phase, a fine and dense microstructure and optimal orientation effect and vanadium refinement effect, and is free of segregation. The minimum primary dendrite arm spacing and the secondary dendrite arm spacing of the alloy columnar crystal are 220  $\mu\text{m}$  and 20  $\mu\text{m}$ , respectively, which are reduced by 52.38% and 44.45%, respectively, compared with those of the high-boron vanadium-free high-speed steel.

In summary, by means of the directional solidification process, the grain orientation of the solidified microstructure can be better controlled such that the high-speed steel presents a certain orientation and has a continuous columnar crystal structure, allowing for greatly improved performance compared with the ordinary high-boron high-speed steel.

The technical solutions of the present application will be further described in detail below with reference to the accompanying drawings and embodiments.

#### BRIEF DESCRIPTION OF THE DRAWINGS

FIG. 1 schematically depicts a directional solidification device according to an embodiment of the present disclosure;

FIGS. 2a-2f shows optical microscopy (OM) topographic images of directionally solidified high-boron high-vanadium high-speed steels containing different levels of vanadium, where (a): 0 wt. % V under lower magnification; (b): 1 wt. % V under lower magnification; (c): 2 wt. % V under lower magnification; (d): 0 wt. % V under higher magnification; (e): 1 wt. % V under higher magnification; and (f): 2 wt. % V under higher magnification;

FIG. 3 shows statistical results of a primary dendrite arm spacing and a secondary dendrite arm spacing in the presence of different levels of vanadium; and

FIG. 4 shows macro-hardness and bending strength test results of the high-boron high-vanadium high-speed steels varying in the vanadium content.

#### DETAILED DESCRIPTION OF EMBODIMENT

10 The present disclosure provides a directionally solidified high-boron and high-vanadium high-speed steel and a method for preparing the same. The resulting directionally solidified vanadium-containing high-boron high-speed steel has well-oriented hard phase (i.e.,  $\text{M}_2\text{B}$  borides), uniform and dense microstructure, large hardness and high bending strength, and is low-cost, stable, and free of segregation. The method provided herein provides a new idea for developing the wear-resistant high-speed steel.

Provided herein is a directionally solidified high-boron 20 high-vanadium high-speed steel, consisting of 0.35-0.48% by weight of C, 1.77-1.82% by weight of B, 4.76-4.81% by weight of Cr, 0.58-0.73% by weight of Si, 0.64-0.90% by weight of Mn, 1.19-1.23% by weight of W, 0.63-0.67% by weight of Mo, 0.06-0.10% by weight of Ti, 0.59-0.61% by weight of Al, 1.88-2.30% by weight of V, and Fe and trace impurities.

25 The directionally solidified high-boron and high-vanadium high-speed steel includes a metal substrate and a hard-phase boride distributed on the metal substrate. Vanadium significantly contributes to the wear resistance and red hardness of high-speed steel materials, and is a strong carbide forming element. The vanadium in the high-speed steel is partially dissolved in the matrix, and partly forms a carbide with high hardness and high thermal stability. The 30 increase of vanadium content is accompanied by the change of the boride in the alloy from rod-like to multi-granular, and continuous decline in the primary dendrite arm spacing and the secondary dendrite arm spacing of the columnar crystal of the directionally solidified alloy matrix.

35 40 When the vanadium content is 2.05 wt. %, the alloy has an evenly distributed hard phase and a fine structure without segregation, and shows the best orientation effect and vanadium refinement effect. The minimum primary dendrite arm spacing and the secondary dendrite arm spacing of the alloy 45 columnar crystal are 220  $\mu\text{m}$  and 20  $\mu\text{m}$ , respectively, which are reduced by 52.38% and 44.45%, respectively, compared with those of the high-boron vanadium-free high-speed steel.

45 The hardness test results demonstrate that the bulk hardness of the alloy increases with the increase of vanadium content. In particular, in the presence of 2.05 wt. % vanadium, the bulk hardness of the steel in the growth plane of the borides (namely  $\text{M}_2\text{B}$  boride (002) plane as its preferred growth plane) reaches the maximum 62.1 HRC, which is 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425

As an important addition element in high-boron high-speed steels, boron mainly plays a key role in forming various high-hardness and high-thermal stability borides with alloying elements. At the same time, the hardenability of the alloy can be enhanced under the dissolution of a slight amount of boron in the substrate. In the presence of 1.77-1.82 wt. % of boron, the microstructure is allowed to have better performance.

A method for preparing the directionally solidified high-speed steel is also provided herein, which is specifically described below.

(S1) Raw materials are subjected to smelting in a furnace to obtain a liquid steel, which is transferred with a ladle. Then 0.148-0.152 g of aluminum filaments are fed to the bottom of the furnace to perform deoxidation. After that, the liquid steel in the ladle is returned to the furnace and subjected to refining via argon blowing at the bottom of the furnace for 8-15 min to obtain the qualified and clean molten high-boron high-vanadium high speed steel.

In an embodiment, the raw materials in step (S1) include 25.176-25.177% by weight of the scrap steel, 41.850-41.860% by weight of the industrial pure iron, 1.038-1.039% by weight of the ferromanganese, 0.463-0.464% by weight of the ferrosilicon, 4.893-4.894% by weight of the pig iron, 8.520-8.521% of the ferrochromium, 10.899-10.900% by weight of the ferroboron, 1.554-1.555% by weight of the ferrotungsten, 1.121-1.122% by weight of the ferromolybdenum, 4.148-4.149% by weight of the ferrovanadium, and 0.335-0.336% by weight of the ferrotitanium.

In an embodiment, before the casting, the sodium silicate-bonded sand mold is dried at 250-280° C. for 6-8 h to prevent the gas evolution during the casting, avoiding the defects in the casting such as strength decline and pores. In this case, when the liquid steel is poured into the cavity formed by the directional solidification device, the side of the cavity hardly affects the heat dissipation, and finally a strong unidirectional heat dissipation condition is formed from top to bottom.

In an embodiment, the scrap steel, the pig iron and the industrial pure iron, the ferromolybdenum, the ferrochromium, the ferrotungsten, the ferrovanadium, the ferromanganese and the ferrosilicon are fed to a furnace in sequence and molten to obtain a first melt, and this process is accompanied by a series of oxidation reactions, such that levels of individual elements are reduced to a reasonable range. The first melt is transferred to a ladle, and at the same time, the ferroboron, the ferrotitanium are fed to the furnace to be molten, and then the first melt in the ladle is transferred back to the furnace to obtain a second melt, which is then transferred to the ladle. When the second melt in the ladle is close to 1520-1530° C., some aluminum filaments are fed to the bottom of the furnace to perform deoxidization, and then the second melt is transferred back to the furnace, and subjected to refining by argon blowing at the bottom of the furnace. By means of the refining and standing, the impurities, oxides and other inclusions in the liquid steel are removed, further improving the refining degree and purity of the liquid steel, eliminating the casting defects and controlling the metallurgical quality.

In an embodiment, the smelting process is performed at 1580-1600° C., higher than the melting point of iron 1534° C., so that the raw materials can be molten rapidly to enable the full stirring and melting, facilitating enhancing the refinement quality.

(S2) The liquid steel obtained in step (S1) is subjected to superheating treatment at 1510-1520° C. with a superheating degree of 49.8-50.2° C., and poured into the directional

solidification device, where a top end of the casting riser of the directional solidification device is spread with high-purity perlite. After cooled to room temperature, the resulting solidified product is subjected to mold dismantling, shakeout, wire cutting, and finishing to obtain the finished high-speed steel product.

In an embodiment, the overheating treatment is performed at 1510-1520° C. (higher than the melting point of iron) for 10-12 min such that the melt can stay liquid and can be mixed completely, enabling the uniform distribution of elements and avoiding segregation.

In an embodiment, the coating layer of the casting mould is 0.8-1.1 mm in thickness, which can mitigate the thermal impact of the high-temperature liquid steel on the casting mould and reduce the internal stress of the arm, preventing the casting from cracking. Moreover, the coating layer with such thickness can also play a role in improving the heat insulation and the filling performance of the casting mold.

In an embodiment, the casting temperature is 1410-1440° C., higher than the liquidus temperature (1381° C.) in the phase diagram of the Fe-B alloy, which can maintain certain superheat to ensure high quality casting.

Before casting, skimming and deoxidation are performed, and an insulation agent (high-purity perlite) is spread uniformly on the insulating riser of the directional solidification device. The solidification is performed at a cooling rate of 12.1-12.3° C./s for 19.0-21.0 s to ensure the good filling capacity, excellent feeding conditions and easy healing of the thermal crack, such that the obtained casting is dense and sound.

In the directional solidification device, four lateral thermal-couples are built into the same level 5 mm away from the bottom of the cold end, and a cooling system formed by embedding a small square copper block in the bottom of the square pure iron. The square pure iron is 300 mm×300 mm×300 mm in size, and the built-in copper block is 150 mm×150 mm×200 mm in size arranged at the bottom centerline 100 mm away from the top surface of the pure iron. The pure iron is closely matched with the copper block, which improves the cooling rate of the casting such that the casting obtains the necessary temperature gradient to form an ideal directional solidification columnar crystal structure.

To render objects, technical solutions and advantages of the embodiments of the present disclosure clearer, the technical solutions of the present application will be clearly and completely described below with reference to the drawings of the embodiments. Obviously, described below are only some embodiments of the present application. The components of the embodiments typically illustrated in the drawings may be arranged and designed in different configurations. Accordingly, the following detailed description of the embodiments illustrated in the drawings is not intended to limit the scope of the application, but merely illustrative of the selected embodiments. Based on the embodiments provided herein, other embodiments obtained by those skilled in the art without paying any creative effort shall fall within the scope of this application.

#### Example 1

The raw material for the preparation of a directionally solidified high-speed steel included 25.176% by weight of a scrap steel, 41.852% by weight of an industrial pure iron, 1.038% by weight of a ferromanganese, 0.463% by weight of a ferrosilicon, 4.893% by weight of a pig iron, 8.520% by weight of a ferrochromium, 10.900% by weight of a ferroboron, 1.554% by weight of a ferrotungsten, 1.121% by

weight of a ferromolybdenum, 4.148% by weight of a ferrovanadium, and 0.335% by weight of a ferrotitanium.

The scrap steel was composed of 0.300% by weight of C, 0.300% by weight of Si, 0.500% by weight of Mn, and Fe. The industrial pure iron was composed of 0.003% by weight of C, 0.020% by weight of Si, 0.150% by weight of Mn, and Fe. The ferromanganese was composed of 6.410% by weight of C, 1.630% by weight of Si, 65.900% by weight of Mn, and Fe. The ferrosilicon was composed of 0.100% by weight of C, 73.100% by weight of Si, and Fe. The pig iron was composed of 4.270% by weight of C, 0.900% by weight of Si, 0.113% by weight of Mn, and Fe. The ferrochromium was composed of 0.240% by weight of C, 59.000% by weight of Cr, 1.700% by weight of Si, and Fe. The ferroboron was composed of 0.320% by weight of C, 0.760% by weight of Si, 18.150% by weight of B, and Fe. The ferrotungsten was composed of 0.060% by weight of C, 0.290% by weight of Si, 0.160% by weight of Mn, 78.507% by weight of W, and Fe. The ferromolybdenum was composed of 0.034% by weight of C, 0.750% by weight of Si, 62.597% by weight of Mo, and Fe. The ferrovanadium was composed of 0.310% by weight of C, 1.010% by weight of Si, 51.896% by weight of V, and Fe. The ferrotitanium was composed of 0.002% by weight of C, 0.015% by weight of Si, 30.009% by weight of Ti, and Fe.

The directionally solidified high-boron high-vanadium high-speed steel was prepared as follows.

(S1) The scrap steel, the pig iron, the industrial pure iron, the ferromolybdenum, the ferrochromium, the ferrotungsten, the ferrovanadium, the ferromanganese and the ferrosilicon were fed to a furnace in sequence and molten to obtain a first melt, which was transferred to a ladle. When the furnace was heated to 1550° C., the ferroboron and ferrotitanium were fed to the furnace and molten, and the first melt in the ladle was transferred back to the furnace to obtain a second melt, which was then transferred to the ladle. After that, 0.148 g of aluminum filament was fed to a bottom of the furnace to perform deoxidization, and then the second melt in the ladle was transferred back to the furnace and subjected to refinement by argon blowing at the bottom of the furnace for 10 min to obtain a liquid steel, which was confirmed to be qualified and clean. Subsequently, the liquid steel was subjected to superheating treatment at 1510° C. for 10 min with a superheating degree of 49.8° C. Before casting, the sodium silicate-bonded sand mold was dried at 250° C. for 6 h.

(S2) The liquid steel obtained in step (S1) was poured into the directional solidification device at a temperature of 1420° C. for directional solidification, where the temperature measurement was enabled by means of a thermal couple, and a chilling block formed by embedding a copper block in a pure iron was employed for cooling; and a thickness of a coating layer was 0.8 mm. Before the casting, skimming and deoxidation were performed, and a thermal insulation agent (high-purity perlite) was spread uniformly on the casting riser of the directional solidification device. The solidification was performed at a cooling rate of 12.1° C./s for 19.0 s. After cooled to room temperature, the resulting solidified product was subjected to mold dismantling, shakeout, wire cutting, and finishing to obtain the directionally solidified high-boron and high-vanadium high-speed steel.

#### Example 2

The raw material for the preparation of a directionally solidified high-speed steel included 25.176% by weight of a

scrap steel, 41.852% by weight of an industrial pure iron, 1.038% by weight of a ferromanganese, 0.463% by weight of a ferrosilicon, 4.893% by weight of a pig iron, 8.520% by weight of a ferrochromium, 10.899% by weight of a ferroboron, 1.554% by weight of a ferrotungsten, 1.121% by weight of a ferromolybdenum, 4.148% by weight of a ferrovanadium, and 0.335% by weight of a ferrotitanium.

The scrap steel was composed of 0.300% by weight of C, 0.300% by weight of Si, 0.500% by weight of Mn, and Fe. The industrial pure iron was composed of 0.300% by weight of C, 0.020% by weight of Si, 0.150% by weight of Mn, and the Fe. The ferromanganese was composed of 6.410% by weight of C, 1.630% by weight of Si, 65.900% by weight of Mn, and Fe. The ferrosilicon was composed of 0.100% by weight of C, 73.100% by weight of Si, and Fe. The pig iron was composed of 4.270% by weight of C, 0.900% by weight of Si, 0.113% by weight of Mn, and Fe. The ferrochromium was composed of 0.240% by weight of C, 58.809% by weight of Cr, 1.700% by weight of Si, and Fe. The ferroboron was composed of 0.320% by weight of C, 0.760% by weight of Si, 18.554% by weight of B, and Fe. The ferrotungsten was composed of 0.060% by weight of C, 0.290% by weight of Si, 0.160% by weight of Mn, 79.150% by weight of W, and Fe. The ferromolybdenum was composed of 0.034% by weight of C, 0.750% by weight of Si, 62.914% by weight of Mo, and Fe. The ferrovanadium was composed of 0.310% by weight of C, 1.010% by weight of Si, 52.020% by weight of V, and Fe. The ferrotitanium was composed of 0.002% by weight of C, 0.015% by weight of Si, 3.167% by weight of Ti, and Fe.

The directionally solidified high-speed steel was prepared as follows.

(S1) The scrap steel, the pig iron, the industrial pure iron, the ferromolybdenum, the ferrochromium, the ferrotungsten, the ferrovanadium, the ferromanganese and the ferrosilicon were fed to a furnace in sequence and molten to obtain a first melt, which was transferred to a ladle. When the furnace was heated to 1560° C., the ferroboron and ferrotitanium were fed to the furnace and molten, and the first melt in the ladle was transferred back to the furnace to obtain a second melt, which was then transferred to the ladle. After that, 0.149 g of the aluminum filament was fed to a bottom of the furnace to perform deoxidization, and then the second melt in the ladle was transferred back to the furnace and subjected to refinement by argon blowing at the bottom of the furnace for 8 min to obtain a liquid steel, which was confirmed to be qualified and clean. Subsequently, the liquid steel was subjected to superheating treatment at 1510° C. for 10 min with a superheating degree of 49.8° C. Before casting, the sodium silicate-bonded sand mold was dried at 260° C. for 6 h.

(S2) The liquid steel obtained in step (S1) was poured into the directional solidification device at a temperature of 1425° C. for directional solidification, where the temperature measurement was enabled by means of a thermal couple, and a chilling block formed by embedding a copper block in a pure iron was employed for cooling; and a thickness of a coating layer was 0.9 mm. Before the casting, skimming and deoxidation were performed, and a thermal insulation agent (high-purity perlite) was spread uniformly on the casting riser of the directional solidification device. The solidification was performed at a cooling rate of 12.1° C./s for 19.5 s. After cooled to room temperature, the resulting solidified product was subjected to mold dismantling, shakeout, wire cutting, and finishing to obtain the directionally solidified high-boron and high-vanadium high-speed steel.

## 11

## Example 3

The raw material for the preparation of a directionally solidified high-speed steel included 25.176% by weight of a scrap steel, 41.851% by weight of an industrial pure iron, 1.038% by weight of a ferromanganese, 0.463% by weight of a ferrosilicon, 4.893% by weight of a pig iron, 8.521% by weight of a ferrochromium, 10.899% by weight of a ferroboron, 1.554% by weight of a ferrotungsten, 1.121% by weight of a ferromolybdenum, 4.148% by weight of a ferrovanadium, and 0.336% by weight of a ferrotitanium.

The scrap steel was composed of 0.300% by weight of C, 0.300% by weight of Si, 0.500% by weight of Mn, and Fe. The industrial pure iron was composed of 0.300% by weight of C, 0.020% by weight of Si, 0.150% by weight of Mn, and the Fe. The ferromanganese was composed of 6.410% by weight of C, 1.630% by weight of Si, 65.900% by weight of Mn, and Fe. The ferrosilicon was composed of 0.100% by weight of C, 73.100% by weight of Si, and Fe. The pig iron was composed of 4.270% by weight of C, 0.900% by weight of Si, 0.113% by weight of Mn, and Fe. The ferrochromium was composed of 0.240% by weight of C, 59.000% by weight of Cr, 1.700% by weight of Si, and Fe. The ferroboron was composed of 0.320% by weight of C, 0.760% by weight of Si, 18.146% by weight of B, and Fe. The ferrotungsten was composed of 0.060% by weight of C, 0.290% by weight of Si, 0.160% by weight of Mn, 79.150% by weight of W, and Fe. The ferromolybdenum was composed of 0.034% by weight of C, 0.750% by weight of Si, 61.000% by weight of Mo, and Fe. The ferrovanadium was composed of 0.310% by weight of C, 1.010% by weight of Si, 52.020% by weight of V, and Fe. The ferrotitanium was composed of 0.002% by weight of C, 0.015% by weight of Si, 26.460% by weight of Ti, and Fe.

The directionally solidified high-speed steel was prepared as follows.

(S1) The scrap steel, the pig iron, the industrial pure iron, the ferromolybdenum, the ferrochromium, the ferrotungsten, the ferrovanadium, the ferromanganese and the ferrosilicon were fed to a furnace in sequence and molten to obtain a first melt, which was transferred to a ladle. When the furnace was heated to 1570° C., the ferroboron and ferrotitanium were fed to the furnace and molten, and the first melt in the ladle was transferred back to the furnace to obtain a second melt, which was then transferred to the ladle. After that, 0.15 g of the aluminum filament was fed to a bottom of the furnace to perform deoxidization, and then the second melt in the ladle was transferred back to the furnace and subjected to refinement by argon blowing at the bottom of the furnace for 12 min to obtain a liquid steel, which was confirmed to be qualified and clean. Subsequently, the liquid steel was subjected to superheating treatment at 1510° C. for 10 min with a superheating degree of 50° C. Before casting, the sodium silicate-bonded sand mold was dried at 265° C. for 7 h.

(S2) The liquid steel obtained in step (S1) was poured into the directional solidification device at a temperature of 1430° C. for directional solidification, where the temperature measurement was enabled by means of a thermal couple, and a chilling block formed by embedding a copper block in a pure iron was employed for cooling; and a thickness of a coating layer was 0.8-1.1 mm. Before the casting, skimming and deoxidation were performed, and a thermal insulation agent (high-purity perlite) was spread uniformly on the casting riser of the directional solidification device. The solidification was performed at a cooling rate of 12.2° C./s for 20.0 s. After cooled to room temperature, the

## 12

resulting solidified product was subjected to mold dismantling, shakeout, wire cutting, and finishing to obtain the directionally solidified high-boron and high-vanadium high-speed steel.

## Example 4

The raw material for the preparation of a directionally solidified high-speed steel included 25.176% by weight of a scrap steel, 41.850% by weight of an industrial pure iron, 1.038% by weight of a ferromanganese, 0.464% by weight of a ferrosilicon, 4.894% by weight of a pig iron, 8.520% by weight of a ferrochromium, 10.899% by weight of a ferroboron, 1.554% by weight of a ferrotungsten, 1.121% by weight of a ferromolybdenum, 4.148% by weight of a ferrovanadium, and 0.336% by weight of a ferrotitanium.

The scrap steel was composed of 0.300% by weight of C, 0.300% by weight of Si, 0.500% by weight of Mn, and Fe. The industrial pure iron was composed of 0.300% by weight of C, 0.020% by weight of Si, 0.150% by weight of Mn, and Fe. The ferromanganese was composed of 6.410% by weight of C, 1.630% by weight of Si, 65.900% by weight of Mn, and Fe. The ferrosilicon was composed of 0.100% by weight of C, 73.100% by weight of Si, and the weight of Fe. The pig iron was composed of 4.270% by weight of C, 0.900% by weight of Si, 0.113% by weight of Mn, and Fe. The ferrochromium was composed of 0.240% by weight of C, 59.300% by weight of Cr, 1.700% by weight of Si, and Fe. The ferroboron was composed of 0.320% by weight of C, 0.760% by weight of Si, 18.350% by weight of B, and Fe. The ferrotungsten was composed of 0.060% by weight of C, 0.290% by weight of Si, 0.160% by weight of Mn, 78.507% by weight of W, and Fe. The ferromolybdenum was composed of 0.034% by weight of C, 0.750% by weight of Si, 60.097% by weight of Mo, and Fe. The ferrovanadium was composed of 0.310% by weight of C, 1.010% by weight of Si, 49.739% by weight of V, and Fe. The ferrotitanium was composed of 0.002% by weight of C, 0.015% by weight of Si, 31.954% by weight of Ti, and Fe.

The directionally solidified high-speed steel was prepared as follows.

(S1) The scrap steel, the pig iron, the industrial pure iron, the ferromolybdenum, the ferrochromium, the ferrotungsten, the ferrovanadium, the ferromanganese and the ferrosilicon were fed to a furnace in sequence and molten to obtain a first melt, which was transferred to a ladle. When the furnace was heated to 1580° C., the ferroboron and ferrotitanium were fed to the furnace and molten, and the first melt in the ladle was transferred back to the furnace to obtain a second melt, which was then transferred to the ladle. After that, 0.151 g of the aluminum filament was fed to a bottom of the furnace to perform deoxidization, and then the second melt in the ladle was transferred back to the furnace and subjected to refinement by argon blowing at the bottom of the furnace for 14 min to obtain a liquid steel, which was confirmed to be qualified and clean. Subsequently, the liquid steel was subjected to superheating treatment at 1510° C. for 12 min with a superheating degree of 50.1° C. Before casting, the sodium silicate-bonded sand mold was dried at 270° C. for 8 h.

(S2) The liquid steel obtained in step (S1) was poured into the directional solidification device at a temperature of 1435° C. for directional solidification, where the temperature measurement was enabled by means of a thermal couple, and a chilling block formed by embedding a copper block in a pure iron was employed for cooling; and a thickness of a coating layer was 1.0 mm. Before the casting,

skimming and deoxidation were performed, and a thermal insulation agent (high-purity perlite) was spread uniformly on the casting riser of the directional solidification device. The solidification was performed at a cooling rate of 12.3° C./s for 21.0 s. After cooled to room temperature, the resulting solidified product was subjected to mold dismantling, shakeout, wire cutting, and finishing to obtain the directionally solidified high-boron and high-vanadium high-speed steel.

#### Example 5

The raw material for the preparation of a directionally solidified high-speed steel included 25.176% by weight of a scrap steel, 41.850% by weight of an industrial pure iron, 1.038% by weight of a ferromanganese, 0.464% by weight of a ferrosilicon, 4.894% by weight of a pig iron, 8.521% by weight of a ferrochromium, 10.899% by weight of a ferroboron, 1.554% by weight of a ferrotungsten, 1.121% by weight of a ferromolybdenum, 4.148% by weight of a ferrovanadium, and 0.335% by weight of a ferrotitanium.

The scrap steel was composed of 0.300% by weight of C, 0.300% by weight of Si, 0.500% by weight of Mn, and Fe. The industrial pure iron was composed of 0.300% by weight of C, 0.020% by weight of Si, 0.150% by weight of Mn, and Fe. The ferromanganese was composed of 6.410% by weight of C, 1.630% by weight of Si, 65.900% by weight of Mn, and Fe. The ferrosilicon was composed of 0.100% by weight of C, 73.100% by weight of Si, and Fe. The pig iron was composed of 4.270% by weight of C, 0.900% by weight of Si, 0.113% by weight of Mn, and Fe. The ferrochromium was composed of 0.240% by weight of C, 59.300% by weight of Cr, 1.700% by weight of Si, and Fe. The ferroboron was composed of 0.320% by weight of C, 0.760% by weight of Si, 18.350% by weight of B, and Fe. The ferrotungsten was composed of 0.060% by weight of C, 0.290% by weight of Si, 0.160% by weight of Mn, 77.840% by weight of W, and Fe. The ferromolybdenum was composed of 0.034% by weight of C, 0.750% by weight of Si, 61.000% by weight of Mo, and Fe. The ferrovanadium was composed of 0.310% by weight of C, 1.010% by weight of Si, 52.020% by weight of V, and Fe. The ferrotitanium was composed of 0.002% by weight of C, 0.015% by weight of Si, 26.460% by weight of Ti, and Fe.

The directionally solidified high-speed steel was prepared as follows.

(S1) The scrap steel, the pig iron, the industrial pure iron, the ferromolybdenum, the ferrochromium, the ferrotungsten, the ferrovanadium, the ferromanganese and the ferrosilicon were fed to a furnace in sequence and molten to obtain a first melt, which was transferred to a ladle. When the furnace was heated to 1600° C., the ferroboron and ferrotitanium were fed to the furnace and molten, and the first melt in the ladle was transferred back to the furnace to obtain a second melt, which was then transferred to the ladle. After that, 0.152 g of the aluminum filament was fed to a bottom of the furnace to perform deoxidation, and then the second melt in the ladle are transferred back to the furnace and subjected to refinement by argon blowing at the bottom of the furnace for 15 min to obtain a liquid steel, which was confirmed to be qualified and clean. Subsequently, the liquid steel was subjected to superheating treatment at 1510° C. for 12 min with a superheating degree of 50.2° C. Before casting, the sodium silicate-bonded sand mold was dried at 280° C. for 8 h.

(S2) The liquid steel obtained in step (S1) was poured into the directional solidification device at a temperature of

1440° C. for directional solidification, where the temperature measurement was enabled by means of a thermal couple, and a chilling block formed by embedding a copper block in a pure iron was employed for cooling; and a thickness of a coating layer was 1.1 mm. Before the casting, skimming and deoxidation were performed, and a thermal insulation agent (high-purity perlite) was spread uniformly on the casting riser of the directional solidification device. The solidification was performed at a cooling rate of 12.3° C./s for 21.0 s. After cooled to room temperature, the resulting solidified product was subjected to mold dismantling, shakeout, wire cutting, and finishing to obtain the directionally solidified high-boron and high-vanadium high-speed steel.

Referring to an embodiment of the directional solidification device illustrated in FIG. 1, four lateral built-in thermocouples were arranged in the same level 5 mm away from the bottom of the cold end for temperature measurement, and a composite cooling system formed by a pure iron block and a small copper block embedded in the bottom thereof was employed. The pure iron block was 300 mm×300 mm×300 mm in size, and the copper block was 150 mm×150 mm×200 mm in size and arranged in the pure iron block with the bottom centerline 100 mm away from the top surface of the pure iron. The pure iron was closely fitted with the copper block, which improves the cooling rate of the casting and facilitates the formation of an ideal directionally solidified columnar crystal structure under a desired temperature gradient.

As shown in FIGS. 2a-f, directionally solidified high-boron high-speed steels respectively with 0.00 wt. %, 1.00 wt. % and 2.05 wt. % of V were compared with respect to the optical topography. It could be seen that in the selected three levels of V (0.00 wt. %, 1.00 wt. %, and 2.05 wt. %), the substrate exhibited an obvious columnar crystal structure growing along the direction of heat flow, and thus the resulting alloy products all had good orientation effect. In the presence of 2.05 wt. % V, the alloy had an evenly distributed hard phase and a fine structure without segregation, and reached the optimal orientation effect and vanadium refinement effect.

Referring to FIG. 3, with respect to the columnar crystal matrix (V content<2.05 wt. %), the primary dendrite arm spacing and the secondary arm dendrite spacing decreased with the increase of V content. When the V content was 2.05 wt. %, the minimum primary dendrite arm spacing and secondary dendrite arm spacing of columnar crystal were 220 μm and 20 μm, respectively, which were reduced by 52.38% and 44.45%, respectively, compared with those of the high-boron vanadium-free high-speed steel.

The primary dendrite arm spacing and the secondary dendrite arm spacing of samples varying in the vanadium level were shown in Table 1.

TABLE 1

| Primary and secondary dendrite arm spacings of steels with different V contents |                                   |                                     |
|---------------------------------------------------------------------------------|-----------------------------------|-------------------------------------|
| V Content (wt. %)                                                               | Primary dendrite arm spacing (μm) | Secondary dendrite arm spacing (μm) |
| 0.00                                                                            | 420                               | 45                                  |
| 1.00                                                                            | 240                               | 25                                  |
| 2.05                                                                            | 220                               | 20                                  |

## 15

The bulk hardness and bending strength of directionally solidified high-boron high-speed steels varying in V content (0.00 wt. %, 1.00 wt. % and 2.05 wt. %) were tested and compared.

Referring to FIG. 4, the bulk hardness of the alloy increased with the increase of vanadium content. In particular, in the presence of 2.05 wt. % vanadium, the alloy hardness of the vertical hard phase cylinder reached the maximum 62.1 HRC, which was 13.04% higher than that of the as-cast high-boron high-speed steel, and 35.42% higher than that of the as-cast high-boron high-speed steel bearing 0.4% by weight of C, 2.0% by weight of B, and 1.0% by weight of V (40.1 HRC). At the same time, the toughness of the alloy was improved by 32%. In addition, the bending strength of the alloy was also enhanced with the increase of the vanadium content, and when the vanadium content was 2.05 wt. %, the bending strength of the parallel hard phase cylinder reached the maximum 1724 MPa, which was 12.41% higher than that of the as-cast high-speed steel. The bulk hardness results of steels were shown in Table 2.

TABLE 2

| bulk hardness of cross section of steels with different V contents        |                |
|---------------------------------------------------------------------------|----------------|
| V content (wt. %)                                                         | Hardness (HRC) |
| 0.00                                                                      | 54.0           |
| 1.00                                                                      | 59.6           |
| 2.05                                                                      | 62.1           |
| As-cast high-boron high-speed steel containing 0.4% C, 2.0% B, and 1.0% V | 40.1           |

The test results of bending strength were shown in Table 3.

TABLE 3

| Bending strength of steels with different V contents |                        |
|------------------------------------------------------|------------------------|
| V content (wt. %)                                    | Bending strength (MPa) |
| 0.00                                                 | 1510                   |
| 1.00                                                 | 1560                   |
| 2.05                                                 | 1724                   |

Overall, by using the method provided herein for preparing the directionally solidified high-speed steel, the prepared high-speed steel has a good orientation effect. In the presence of 2.05 wt. %, the obtained alloy has an evenly distributed hard phase, a fine structure without segregation, and shows the best orientation effect and vanadium refinement effect. The minimum primary dendrite arm spacing and the secondary dendrite arm spacing of the alloy columnar crystal are 220  $\mu\text{m}$  and 20  $\mu\text{m}$ , which are reduced by 52.38% and 44.45%, respectively, compared with those of the high-boron vanadium-free high-speed steel. The alloy hardness and the bending strength are increased by 13.04% and 12.41%, respectively. As a result, the directionally solidified high-speed steel provided herein has an evenly distributed hard phase, a fine structure without segregation, and a high hardness and bending strength. The method provided herein is low-cost and offers a new idea for developing the wear-resistant high-speed steel.

In summary, by means of the directional solidification process, the grain orientation of the solidified microstructure can be better controlled such that the high-speed steel presents a certain orientation and has a continuous columnar

## 16

crystal structure, allowing for greatly improved performance compared with the ordinary high-boron high-speed steel.

Described above are merely illustrative of the technical solutions of the present disclosure, and are not intended to limit the present disclosure. It should be understood that all changes, replacements and modifications made by those skilled in the art on the basis of the technical solutions proposed herein without departing from the scope of the disclosure shall fall within the scope of the present disclosure defined by the appended claims.

What is claimed is:

1. A method of preparing a directionally solidified steel, comprising:

(S1) subjecting a raw material to smelting at 1580-1600°

C. and refining to obtain a liquid steel; wherein the raw material comprises pig iron, scrap steel, ferrochromium, ferromanganese, ferroboron, a ferrovanadium, industrially pure iron, ferromolybdenum, ferrotungsten, ferrosilicon and ferrotitanium; and

(S2) subjecting the liquid steel to superheating and directional solidification at a casting temperature of 1420-1430° C. followed by cooling to room temperature to obtain the directionally solidified steel;

wherein the directional solidification is performed in a directional solidification device equipped with a sodium silicate-bonded sand mold as a casting mould; an inner side surface of the sodium silicate-bonded sand mold is coated with an aluminum oxide coating with an average thickness of 0.8-1.1 mm; and

in step (S2), before the directional solidification, the sodium silicate-bonded sand mold is dried at 250-280° C. for 6-8 h.

2. The method of claim 1, wherein in step (S1), the raw material comprises 4.893-4.894% by weight of the pig iron,

25.176-25.177% by weight of the scrap steel, 8.520-8.521% by weight of the ferrochromium, 1.038-1.039% by weight of the ferromanganese, 10.899-10.900% by weight of the ferroboron, 4.148-4.149% by weight of the ferrovanadium, 41.850-41.860% by weight of the industrially pure iron, 1.121-1.122% by weight of the ferromolybdenum, 1.554-1.555% by weight of the ferrotungsten, 0.463-0.464% by weight of the ferrosilicon and 0.335-0.336% by weight of the ferrotitanium.

3. The method of claim 1, wherein in step (S1), the smelting and the refining are performed through steps of:

feeding the scrap steel, the pig iron and the industrial pure iron to a furnace, and then feeding the ferromolybdenum, the ferrochromium, the ferrotungsten, the ferrovanadium, the ferromanganese and the ferrosilicon to the furnace; heating the furnace to 1550-1600° C. to obtain a first melt; transferring the first melt with a ladle;

feeding the ferroboron and the ferrotitanium to the furnace and then transferring the first melt in the ladle back to the furnace to obtain a second melt; transferring the second melt to the ladle; introducing 0.148-0.152 g of an aluminum filament to a bottom of the furnace for deoxidization; transferring the second melt back to the furnace; and performing argon blowing at the bottom of the furnace for 8-15 min for refining.

4. The method of claim 1, wherein in step (S2), the superheating of the liquid steel is performed at 1510-1520° C. for 10-12 min with a superheat degree of 49.8-50.2° C.

5. The method of claim 1, wherein in step (S2), a top end of a casting riser of the directional solidification device is spread with a thermal insulating agent; the directional solidification device is performed at a cooling rate of 12.1-12.3°

C./s for 19.0-21.0 s; and after cooled down to a room temperature, the directionally solidified steel is subjected to mold dismantling, shakeout and wire cutting.

6. The method of claim 5, wherein the directional solidification device adopts a thermal-couple for heating monitor. 5

7. The method of claim 6, wherein the casting mould of the directional solidification device is coated with a coating layer having a thickness of 0.8-1.1 mm.

\* \* \* \* \*